

## UNITED STATES PATENT OFFICE

2,344,392

CRANKCASE LUBRICANT AND CHEMICAL  
COMPOUND THEREFOR

Elmer W. Cook, New York, N. Y., and William D. Thomas, Jr., Stamford, Conn., assignors to American Cyanamid Company, New York, N. Y., a corporation of Maine

No Drawing. Application November 8, 1941,  
Serial No. 418,326

6 Claims. (Cl. 252—48)

This invention relates to a new class of chemical compounds which are useful as addition agents to lubricating oils of the type known as crankcase oil; i. e. hydrocarbon oils of relatively low viscosity and pour point such as are used in the crankcases of internal combustion engines and to lubricating oils of this type containing such additives. More particularly, the invention relates to the heavy metal salts of the dicapryl ester of dithiophosphoric acid and to lubricating oils of the above type containing this class of compounds. By the term "heavy metal salt" in the following specification and claims we mean the salts of the metallic elements of groups II to VIII inclusive of the periodic system and especially such salts as those of the alkaline earth metals magnesium, calcium, strontium and barium and other metals such as zinc, aluminum, chromium, tin, cobalt and nickel which form water-insoluble salts with dicapryl dithiophosphate. Salts of lithium, sodium, potassium, rubidium and caesium, the alkali metals, are excluded from the invention.

The heavy metal salts of dicapryl dithiophosphoric acid ester are water-insoluble but hydrocarbon oil-soluble compounds. Most of the compounds of this class, including all the alkaline earth metal salts are brownish-yellow solids of low melting point, whereas the zinc salt is a viscous liquid at ordinary temperatures. The compounds as a class are soluble in hydrocarbon oils of the type of 10-W grade lubricating oils to the extent of 30-50% by weight, and are therefore well adapted for manufacture and sale in the form of lubricating oil solutions of fairly high concentration, which can be readily blended with further amounts of oil to concentrations of 0.1-3%, in which they are used.

We have discovered that lubricating oils containing 0.1-3% of heavy metal salts of the dicapryl ester of dithiophosphoric acid possess several remarkable and unexpected properties. We have found that these compounds are detergents for the prevention of sludge deposits in truck, bus, aeroplane and marine gasoline and Diesel engines, and that they also possess extremely important non-oxidizing or antioxidant properties when compared with other metal salt detergents that have previously been used. Moreover, these compounds possess a remarkable degree of stability against decomposition and sludge formation under the conditions of heavy duty use in lubricating oil when it is considered that they are esters of aliphatic secondary alcohols of a type that are known to be considerably less heat-

stable than the esters of the corresponding primary alcohols.

Dicapryl dithiophosphoric acid is prepared by reacting capryl alcohol with phosphorous pentasulfide in the ratio of approximately 4 moles of the alcohol for each mole of  $P_2S_5$ , the reaction being carried out by heating the two ingredients together at 80-95° C. with stirring for about 2½ hours. When the evolution of  $H_2S$  has subsided 10 the resulting dicapryl dithiophosphoric acid ester is dissolved in a mixture of absolute alcohol and benzene and sufficient heavy metal oxide is added to effect neutralization. The mixture is heated to complete the neutralization and a part of the 15 solvent is evaporated to expel the water of neutralization, whereupon the solution is filtered and the filtrate evaporated to recover the product. When an alkaline earth metal oxide is used in this manner the alkaline earth metal salts so obtained have the following probable structural 20 formula



The corresponding salts of metals of higher valency, such as the aluminum and chromium salts have similar structural formulas in which three or more thiophosphoric acid ester radicals are linked through sulfur to the metal.

As is noted above one of the most important 35 features of our invention resides in the addition to lubricating oils of the type of hydrocarbon crankcase oils of the heavy metal salts of the above-defined class, either alone or in admixture with other ingredients, in amounts sufficient to exert sludge-dispersing properties under heavy 40 duty service conditions. The formation of sludge in crankcase oils is intimately related to the production of oxidation products of the type of organic acids and it is another important advantage of the heavy metal dicapryl dithiophosphates 45 that they do not cause an increase in oxygen absorption and consequent sludge formation in the oil. Moreover, our new compounds cooperate effectively with the heavy metal salts of di-(2,4- 50 diamyl phenol) monosulfide described in our Patent No. 2,249,626 and with the alkaline earth metal salts of petroleum sulfonates described in our copending application Serial No. 419,016, filed November 13, 1941, either or both of which may 55 be used to combat oxidation and decomposition.

in the lubricating oil, and oils containing the heavy metal dicapryl dithiophosphates in admixture with either or both of these compounds constitute another important feature of our invention.

The invention will be further illustrated in detail by the following specific examples, which present results obtained with a representative heavy metal salt of dicapryl dithiophosphate. It should be understood, however, that the invention in its broader aspects is not limited to these examples.

*Example 1*

260 parts by weight of capryl alcohol



were stirred rapidly with 111 parts by weight of finely ground  $\text{P}_2\text{S}_5$  and heated at 80-95° C. for about 2½ hours. At the end of this time practically all of the  $\text{P}_2\text{S}_5$  was reacted and the dicapryl dithiophosphoric acid remained as a brown liquid. 354 parts by weight of the product so obtained were dissolved in a mixture of equal parts of absolute ethyl alcohol and benzene and stirred rapidly while 77 parts by weight of powdered barium oxide were added to effect neutralization. The mixture was warmed to complete the neutralization and then heated to boiling and a part of the solvent was evaporated to expel the water of neutralization. The solution was then filtered from any traces of barium salts and the filtrate evaporated. The barium dicapryl dithiophosphate was recovered as a brownish-yellow crystalline material of low melting point, insoluble in water but soluble to the extent of about 50% in 10-W grade Pennsylvania (paraffin base) lubricating oil.

The corresponding zinc salt was prepared by adding 41 parts by weight of finely powdered zinc oxide to a solution of 354 parts of dicapryl dithiophosphoric acid in an alcohol-benzene mixture as described above. The product was obtained as a thin oily liquid which was easily soluble in lubricating oil.

*Example 2*

The barium dicapryl dithiophosphate was tested in representative Pennsylvania lubricating oils by an accelerated oxidation test known as the catalytic Indiana test. The testing apparatus consists of a constant temperature bath maintained at 341° F. in which a number of large glass test tubes are immersed. 300 cc. samples of the oil under test are poured into these tubes and air at the rate of 10 liters per hour is

bubbled through the oil. In order to reproduce the conditions existing in the crankcase of an engine weighed strips of copper-lead alloy are suspended in the oil samples. As metallic surfaces, particularly copper, greatly accelerate the rate of oxidation and decomposition of the oil in the presence of oxygen this is an important factor in the test. Bearing corrosion rates can also be determined by again weighing the strips after 70 hours immersion, which is the usual test period.

The results obtained by the above test procedure are shown in the following table, wherein oil A was a solvent refined 10-W grade oil and oil B was a phenol-extracted 10-W grade oil.

|                                        | A. P. I. gravity oxidized oil | Naphtha insoluble | Bearing loss, mg. Cu-Pb | Neut. No. |
|----------------------------------------|-------------------------------|-------------------|-------------------------|-----------|
| 20                                     |                               | Per cent          |                         |           |
| Oil A                                  |                               |                   | 201                     |           |
| Oil A+0.6% Ba dicapryl dithiophosphate |                               |                   | 3                       |           |
| Oil B                                  | 23.5                          | 17.47             | 215                     | 4.68      |
| Oil B+0.4% Ba dicapryl dithiophosphate |                               |                   | +22                     |           |
| Oil B+0.6% Ba dicapryl dithiophosphate | 27.3                          | 3.02              | +16                     | 3.19      |

This application is a continuation-in-part of our copending application, Serial No. 401,960, filed July 11, 1941.

What we claim is:

1. A solution of a heavy metal salt of the dicapryl ester of dithiophosphoric acid in lubricating oil.
2. A solution of an alkaline earth metal salt of the dicapryl ester of dithiophosphoric acid in lubricating oil.
3. A solution of the barium salt of the dicapryl ester of dithiophosphoric acid in lubricating oil.
4. A lubricating oil composition comprising a crankcase oil having dissolved therein 0.1-3% of a heavy metal salt of the dicapryl ester of dithiophosphoric acid.
5. A lubricating oil composition comprising a crankcase oil having dissolved therein 0.1-3% of an alkaline earth metal salt of the dicapryl ester of dithiophosphoric acid.
6. A lubricating oil composition comprising a crankcase oil having dissolved therein 0.1-3% of the barium salt of the dicapryl ester of dithiophosphoric acid.

ELMER W. COOK.

WILLIAM D. THOMAS, JR.